

Patented June 10, 1947

2,422,075

# UNITED STATES PATENT OFFICE

2,422,075

## STABILIZED LUBRICATING EMULSIONS

Malcolm D. Bray, Fishkill, N. Y., assignor to The Texas Company, New York 17, N. Y., a corporation of Delaware

No Drawing. Application August 31, 1944,  
Serial No. 552,203

7 Claims. (Cl. 252—49.5)

1

This invention relates to a stable oil-in-water emulsion and particularly to an emulsified lubricating composition suitable for the lubrication of air compressors and the like.

It has been found that a guanidine salt of a carboxylic acid possessing at least 10 carbon atoms, such as a soap-forming fatty acid, is an efficient emulsifying and thickening agent for oil-in-water emulsions. The oil-in-water emulsions, which are emulsified by the incorporation of small amounts of guanidine stearate, are unusually stable at atmospheric temperatures, but are inclined to separate at elevated temperatures. The addition of the guanidine salt also causes a thickening effect, thereby providing an oil-in-water emulsion of varying consistency, depending upon the amount of guanidine salt used.

Oil-in-water emulsions have been recognized as particularly advantageous in the lubrication of metal surfaces where the temperatures encountered are sufficient to volatilize the lubricating oil. Such temperatures are generally in the range of 500—1000° F. The lubricating emulsions useful for this purpose are particularly the non-metal emulsions, such as disclosed and claimed in U. S. Patent No. 2,353,830, issued to Gus Kaufman, Karl Uhrig, and Robert S. Barnett on July 18, 1944. This patent is directed to an oil-in-water lubricating emulsion in which the emulsifying agent is an alkylolamine soap of a higher fatty acid and the thickening agent is a free fatty acid. The use of this type of emulsion is attended with certain disadvantages in that the presence of the free fatty acid reduces the stability of the emulsion and renders the lubricant corrosive to copper and steel. These corrosive tendencies result in a build-up of deposits and separation of the emulsion which ultimately cause uneven lubrication and seizure of lubricating surfaces.

According to the present invention it has been discovered that an emulsion of an oil in water in which the emulsifying agent consists of the combination of a guanidine salt of a high molecular weight fatty acid and an alkylolamine salt of a carboxylic acid containing at least ten carbon atoms, possesses exceptional stability even at elevated temperatures and over long periods of storage. Stable emulsions of this type are useful for many purposes such as spray bases, insecticide bases, dye baths, flotation oils, cosmetic bases, and the like, but for the purpose of the present invention the following detailed description will be restricted to their application as lubricating emulsions.

2

A lubricating emulsion suited to the lubrication of air compressors and the like, is one which preferably is possessed of the following characteristics: Stability at atmospheric and elevated temperatures, optimum consistency to provide a satisfactory feeding rate, minimum corrosive action on metals used in the lubrication system, minimum residue upon volatilization, and detergent or cleaning action upon carbonaceous deposits formed on lubricating surfaces.

A lubricant which substantially satisfies the above requirement is obtained from an emulsion of mineral oil in water with an emulsifying agent comprising the combination of guanidine stearate and triethanolamine stearate. In the lubrication of air pumps, where the lubricant is in contact with both copper and steel, it is preferable to use an emulsifying combination in which the ratio of the guanidine salt to triethanolamine salt is greater than 1, and to include in the emulsion composition a small amount of free triethanolamine. The effect of the larger proportions of guanidine salt and the addition of free triethanolamine is to obtain a strongly alkaline emulsion which is substantially non-corrosive to copper or steel.

The characteristics of the mineral oil component naturally vary with the type of lubrication required of the emulsion, but in most instances it is preferable to select a low viscosity distillate oil in place of a high viscosity residual oil, due to the lower carbonaceous residues resulting from the volatilization of the distillate oils. For the best results in the lubrication of air compressors a petroleum oil is selected whose viscosity is within the range of 60—100 Saybolt Universal seconds at 210° F. Such an oil may be a single fraction or a mixture of a high and low viscosity oil blended to the desired viscosity.

Although guanidine stearate is specifically set forth as one component of the emulsifying agent, other guanidine salts of higher molecular weight fatty acids may be substituted therefor. Such acids include the fatty acids containing at least 10 carbon atoms, examples of which are lauric, palmitic, myristic, behenic acids and their derivatives, or mixtures thereof. The guanidine salts of unsaturated fatty acids, such as the oleate, are not suitable because of the instability of the resulting emulsions.

In place of triethanolamine stearate other alkylolamine salts of monocarboxylic acids may be used. The alkylolamines include the commercial mixtures of the various ethanolamines and propanol amines, together with their alkylated

derivatives and other aliphatic amines known to be equivalent thereto. The monocarboxylic acids which form the acidic constituent of the alkyloamine salts include the fatty acids and unsaturated fatty acids, such as palmitic and oleic acids and, in general, the aliphatic monocarboxylic acids containing at least ten carbon atoms, together with mixtures thereof, may be used.

As previously mentioned, it has been found desirable to incorporate into the emulsion a small amount of free triethanolamine in order to provide a maximum resistance to corrosion of copper and steel. Here again, other alkyloamines may be substituted therefor, and the usual practice is to incorporate the same alkyloamine as is present in the salt. When the alkyloamine salt is prepared in situ, this is accomplished by adding a calculated quantity of alkyloamine in excess of that required to neutralize the monocarboxylic acid. The proportions of free alkyloamine in the emulsion composition may be as high as 1%, although the best balance between corrosive resistance and stability of the emulsion is obtained with a maximum of 0.5%.

A non-corrosive lubricating emulsion, particularly suited to the lubrication of railway air pumps, may be compounded within the following range of proportions:

|                                                                       | Per cent | 30 |
|-----------------------------------------------------------------------|----------|----|
| Organic salts (ratio of guanidine to alkyloamine salt greater than 1) | 1-15     |    |
| Free alkyloamine                                                      | 0.01-1   |    |
| Mineral oil                                                           | 5-25     |    |
| Water                                                                 | 59-93.99 |    |

These proportionate ranges are predicated upon the composition of the finished emulsion which contains the optimum amount of water. However, this type of emulsion base is not affected by the loss of water and will readily take up water when desired. Furthermore, an emulsion base containing little or no water can be prepared and the required amount of water necessary to yield the desired consistency can be incorporated at the time of use.

An illustration of the preparation of the preferred type of lubricating emulsion can be had from the following example:

2.97 pounds of stearic acid (Saponification No. 210) and approximately 40 pounds of water were charged to a steam-heated kettle which is heated to 180-200° F. and stirred at a fairly rapid rate; 3.5" paddles rotating at 102 R. P. M., giving a peripheral speed of 187 ft. per minute were used. After the temperature was brought up to 180-200° F., 0.80 pound of guanidine carbonate (95% pure), dissolved in a minimum amount of water, were added, with stirring over a period of approximately one hour. The addition of guanidine carbonate results in foaming and frothing of the mixture due to the escaping carbon dioxide. The mixture was then stirred until all the foam had disappeared and the gas had been worked out of the mixture. This stirring operation usually requires approximately one hour in laboratory kettles. Fifteen pounds of a pale oil having a viscosity of 88-92 Saybolt Universal seconds at 210° F., were then added to the mixture as fast as it could be emulsified, which usually requires from 15 to 30 minutes. The mixture was then stirred for approximately 15 minutes in order to make certain that the mineral oil was completely emulsified. 0.703 pound of commercial triethanolamine were dissolved in sufficient water

to make the total added water equal to 80.5% of the finished emulsion, and this solution was then added to the oil-water emulsion over a period of approximately one hour. The temperature must be watched very closely during the addition of the triethanolamine in order to maintain the range of 180-200° F. The stirring rate was then reduced to a peripheral speed of 139 ft. per minute and the mixture allowed to cool to 100° F. or less before drawing. Maintaining the temperature of the mixture at 180° F. or above is imperative until the emulsion is formed, otherwise the guanidine stearate precipitates. Water can be worked in at the drawing temperature, which is 100° F. or less, to compensate for any loss during manufacture. The product, which appears as a light tan homogeneous cream, is then drawn through a suitable straining medium, such as cheese cloth.

Typical analytical results on the lubricating emulsion of the example are as follows:

|                                      | Obtained By Analysis | Theoretical |
|--------------------------------------|----------------------|-------------|
| Guanidine Stearate.....per cent..... | 3.2-3.1              | 2.7         |
| Triethanolamine Stearate.....do..... | 1.2-1.3              | 1.1         |
| Free Triethanolamine.....do.....     | 0.17-0.19            | 0.3         |
| Mineral Oil.....do.....              | 17.2-17.3            | 15.0        |
| Water.....do.....                    |                      | 80.9        |

Obviously many modifications and variations of the invention, as hereinbefore set forth, may be made without departing from the spirit and scope thereof and therefore only such limitations should be imposed as are indicated in the appended claims.

I claim:

1. A lubricating emulsion comprising an emulsion of mineral oil-in-water, a guanidine salt of a soap-forming saturated fatty acid, and an alkyloamine salt of an aliphatic monocarboxylic acid containing at least 10 carbon atoms, said alkyloamine salt being present in amounts sufficient to stabilize said emulsion at elevated temperatures.
2. A lubricating emulsion comprising a viscous emulsion of mineral oil-in-water, said mineral oil being within the viscosity range of 60-100 Saybolt Universal seconds at 210° F., a guanidine salt of a soap-forming saturated fatty acid, an alkyloamine salt of an aliphatic monocarboxylic acid containing at least 10 carbon atoms, and free alkyloamine, said free alkyloamine being present in amounts sufficient to substantially inhibit steel corrosion.
3. A stable emulsion comprising an emulsion of mineral oil in water in which the emulsifying agent is a guanidine salt of a saturated monocarboxylic acid containing at least 10 carbon atoms.
4. A stable emulsion comprising an emulsion of mineral oil in water in which the emulsifying agent is a guanidine salt of a soap-forming saturated fatty acid.
5. An oil-in-water emulsion comprising an emulsion of mineral oil in water in which the emulsifying agent is a combination of a guanidine salt of a saturated fatty acid containing at least 10 carbon atoms, and an alkyloamine salt of a carboxylic acid containing at least 10 carbon atoms, said alkyloamine salt being present in amounts sufficient to stabilize said emulsion at elevated temperatures.
6. A stable emulsion comprising an emulsion of mineral-in-water, a guanidine salt of a soap-

forming saturated fatty acid, and an alkyloamine salt of an aliphatic monocarboxylic acid containing at least 10 carbon atoms, said alkyloamine salt being present in amounts sufficient to stabilize said emulsion at elevated temperatures.

7. A non-corrosive lubricating emulsion comprising an emulsion of mineral oil-in-water, a guanidine salt of a soap-forming saturated fatty acid, an alkyloamine salt of an aliphatic monocarboxylic acid containing at least 10 carbon atoms, and free alkyloamine in which the ratio of the guanidine salt to alkyloamine salt is greater than 1 and in which said free alkyloamine is present in amounts to substantially inhibit steel corrosion.

15 MALCOLM D. BRAY.

REFERENCES CITED

The following references are of record in the file of this patent:

UNITED STATES PATENTS

| Number       | Name      | Date          |
|--------------|-----------|---------------|
| 2,284,086    | Ericks    | May 26, 1942  |
| 2,345,199    | Hodson    | Mar. 28, 1944 |
| 2,174,907    | Waugh     | Oct. 3, 1939  |
| 2,353,830    | Kaufman   | July 18, 1944 |
| 2,349,326    | Wilson    | May 23, 1944  |
| 10 1,830,970 | Sullivan  | Nov. 10, 1931 |
| 2,079,803    | Holtzclaw | May 11, 1937  |
| 2,304,113    | Morgan    | Dec. 8, 1942  |
| 1,848,213    | Weigand   | Mar. 8, 1932  |

OTHER REFERENCES

- 15 Page 159 of vol. II of Gregory's book entitled "Uses and Applications and Related Materials" (1944). (Copy in Div. 64.)
- 20 Pages 382 and 383 of the Organic Chemistry by Fieser and Fieser (1944). (A copy in Div. 64.)